

Jan. 17, 1950

F. W. GIBSON

2,494,806

INFLATED BALL

Filed Dec. 20, 1947

Fig. 1



Fig. 2



Fig. 3



*INVENTOR.*  
Frederick W. Gibson

BY

*Johnson and Kline*  
ATTORNEYS

## UNITED STATES PATENT OFFICE

2,494,806

## INFLATED BALL

Frederick W. Gibson, Chicopee, Mass., assignor to  
 A. G. Spalding & Bros., Inc., Chicopee, Mass.,  
 a corporation of Delaware

Application December 20, 1947, Serial No. 792,987

4 Claims. (Cl. 273—65)

1

The present invention relates to playballs and is particularly adapted to inflated balls such as basketballs and the like which are handled in play and in which a rubber cover is substituted for the usual leather cover thereon.

While the rubber cover produces a less expensive ball which will wear better than a leather cover particularly with out-of-doors use, it possesses the disadvantage particularly when worn in that it becomes slippery when wet so that it is difficult to grasp and handle and also has a feel which is distinctly different from that of leather to which players are accustomed.

Accordingly, it is an object of the present invention to provide a ball having a rubber cover thereon which feels and has the appearance of leather, which is not slippery when wet, and which, as the cover wears down, presents the fibrous feel of worn leather.

This is accomplished by providing in the composition of the rubber cover for the ball short, relatively stiff textile fibers. These fibers, as the ball wears down, project minutely above the surface of the ball to give the fibrous feel of worn leather. They also produce a surface which resists slipping of the ball in the hand when it is wet.

It has been found that in order to secure best results clean short fibers of wool, cotton or rayon be mixed into the cover stock as it is compounded and then molded on the ball. The present preferred composition, however, is made from scrap tennis ball cover stock which is ground up very finely. This stock is made up of felted relatively stiff wool fibers and has normally a small amount of rubber cement on one surface thereof which it has been found aids the dispersion of the fiber in the cover stock.

Other features and advantages of the invention will be apparent from the specification and claims when considered in connection with the drawings in which:

Figure 1 shows a section of the ball showing the cover positioned on the carcass.

Fig. 2 is an enlarged sectional view of the cover showing the relation of the fibers therein when the ball is molded.

Fig. 3 shows a sectional view of the ball as the cover becomes slightly worn.

As shown in the drawings the ball comprises a carcass 10 of textile fabric, which may be rendered impervious to air and used as a bladder or which may be provided with a separate bladder 11 as shown. The carcass is provided with a rubber molded cover 12 of cover material made in accordance with the present invention.

In compounding the cover material there is mixed into the rubber, in addition to a filler, accelerators and vulcanizing agents, a quantity of relatively short fibers indicated at 13 which are

2

thoroughly disposed throughout. These fibers, in the preferred form of the invention comprise ground-up scraps from the material used in making tennis ball covers. This material is made from relatively stiff wool felt and is coated on one side with a rubber adhesive by which the cover sections cut therefrom are adhered to the rubber center of the tennis ball. After the covers are cut, the scrap which is left over is ground very fine and the fibers thus produced. These fibers which have a small quantity of rubber cement thereon, are incorporated into the rubber compound and dispersed through it. It has been found that the small amount of rubber on these fibers aids in their uniform dispersion through the mix. After the cover stock is compounded, it is preferably calendered and applied in sections to the carcass. The covered carcass is placed in a mold which is usually provided with indentations and grooves to produce a pebble grain finish and simulated seams in the finished cover so that its outward appearance is substantially that of a leather cover and it has the feel of smooth finished leather.

It will be noted in Fig. 2 that the fibers are dispersed throughout the cover but do not project beyond the molded surface.

The pebbled surface provides sufficient grip for a rubber covered ball when it is new but as this surface wears down the effect of the pebbles diminishes and the rubber becomes slippery particularly when the hands or ball are wet. However, with the cover of the present invention this difficulty is overcome for as soon as the pebbles on the cover start to wear down the fibers project slightly above the ball surface as shown at 13a in Fig. 3. The fibers projecting from the surface provide the ball with the fibrous feel of worn leather and produces a gripping surface for the rubber cover which is resistant to slipping even when the ball or hands are wet.

One recipe for the cover composition which has been highly successful is as follows:

| Material                                    | Parts      |
|---------------------------------------------|------------|
| Rubber                                      | 100.00     |
| Zinc Oxide                                  | 5.00       |
| Stearic Acid                                | 1.00       |
| Anti-Oxidant                                | 1.00       |
| Filler (clay)                               | 25.00      |
| Fibrous Material (Shoddy, Felt Scrap, etc.) | 20.00      |
| Accelerator                                 | 1.00       |
| Booster                                     | 0.25       |
| Sulphur                                     | 3.00       |
| Color                                       | As desired |

It is to be understood, however, that the proportions of the rubber, filler, accelerators and vulcanizing agents may be varied slightly to produce the desired effect and color and the amount of fibrous material may be varied as required to produce the desired feel.

In lieu of the ground tennis cover stock embodied in the composition, ground felt scrap, shoddy, or short wool, cotton or rayon fibers may be used. When ordinary mill shoddy is employed it must be thoroughly cleaned for it has been discovered that such shoddy contains many greases and dirt which accumulate on the fibers during the weaving process which detract from the mechanical qualities and feel of the cover.

Variations and modifications may be made within the scope of this invention and portions of the improvements may be used without others.

I claim:

1. An inflated playball having a fabric carcass and a molded rubber cover thereon, said cover including short textile fibers therein to project therefrom as the cover wears down to provide a fibrous surface which is resistant to slipping in the hands when the ball or hands are wet and having a feel of leather. 15

2. An inflated playball having a fabric carcass and a molded rubber cover thereon, said cover having a pebbled surface formed thereon and including short textile fibers therein to project therefrom as the pebbled surface wears down to provide a fibrous surface which is resistant to slipping in the hands when the ball or hands are wet and having a feel of leather. 25

3. An inflated playing ball having a base and a molded rubber cover thereon, said cover including ground fibrous tennis ball cover scrap containing short textile fibers to project from the surface when the surface is worn.

4. An inflated playing ball having a fabric carcass and a molded rubber cover thereon, said covering including ground fibrous tennis ball cover scrap containing short textile fibers, said ground scrap projecting from said surface as the cover wears and producing a feel similar to that of worn leather.

FREDERICK W. GIBSON.

#### REFERENCES CITED

The following references are of record in the file of this patent:

#### UNITED STATES PATENTS

| 20 | Number    | Name | Date           |
|----|-----------|------|----------------|
|    | 2,295,815 | Webb | Sept. 15, 1942 |

#### FOREIGN PATENTS

| Number | Country | Date                             |
|--------|---------|----------------------------------|
| 25     | 429,438 | Great Britain ----- May 28, 1935 |